

Aug. 27, 1968

E. W. EVANS ET AL

3,399,059

TITANIUM ALLOYS

Filed June 14, 1965

2 Sheets-Sheet 1



FIG. 1.

INVENTORS

EVAN WILLIAM EVANS  
MICHAEL DUNCAN SMITH

By  
Cochrane, Clegg & Cochran  
ATTORNEYS

Aug. 27, 1968

E. W. EVANS ET AL.

3,399,059

TITANIUM ALLOYS

Filed June 14, 1965

2 Sheets-Sheet 2



FIG. 2.

INVENTORS  
EVAN WILLIAM EVANS  
MICHAEL DUNCAN SMITH

By *Cochrane, Abeling & Cochran*  
ATTORNEYS

1

3,399,059

## TITANIUM ALLOYS

Evan William Evans, Hagley, and Michael Duncan Smith, Shenstone, Lichfield, England assignors to Imperial Metal Industries (Kynoch) Limited, London, England, a corporation of Great Britain

Filed June 14, 1965, Ser. No. 463,573

Claims priority, application Great Britain, June 23, 1964,

25,932/64

10 Claims. (Cl. 75—175.5)

### ABSTRACT OF THE DISCLOSURE

Titanium-base alloys consisting of 15—35% molybdenum, 15—35% vanadium with the total molybdenum plus vanadium content being in the range 40—55% have high stress rupture life at high temperature. The properties of the basic alloy are improved by the addition of hafnium, boron and carbon.

This invention relates to titanium alloys containing substantial quantities of the beta stabilising elements molybdenum and vanadium and possessing a stable all-beta structure. The alloys combine high creep strength at elevated temperatures with good room temperature strength and adequate ductility.

Accordingly the present invention provides a titanium alloy containing 15—35% molybdenum, 15—35% vanadium, the total molybdenum plus vanadium content being in the range 40—55%, 0.01—0.2 boron, balance titanium apart from impurities. The presence of boron in the alloys of the present invention confers good creep properties and a further increase in creep strength is obtained by additions of 0.1—5% hafnium and 0.01—0.2% carbon.

Zirconium up to 8% preferably in the range 4—8% may be added to these alloys to strengthen them and to raise the recrystallisation temperature by 75° C. or more and also to modify oxidation resistance. A content of 5% has been found to be satisfactory.

Incidental alloying elements, that is those elements which are well known in titanium metallurgy and which may be added in small quantities to the alloys of the present invention without adversely affecting their properties, may be present. Examples of such elements are 0—5% tungsten, tantalum, niobium and chromium to modify the strength and 0—5% chromium, and aluminium to modify oxidation resistance.

Tungsten and niobium are the best of such elements for strengthening the alloys and tungsten may with advantage be added up to 10%, as shown in Table I.

Typical impurities are up to 0.5% each of silicon and iron, derived from the starting vanadium, up to 0.3% of oxygen and up to 0.1% each of nitrogen and carbon.

Alloys in accordance with the present invention include aircraft engines within their field of application. As is well known, density plays an important part in the choice of materials for use in aircraft and alloys herein described have a favourable density with which are combined good elevated temperature properties and good fabricability.

It is necessary that sufficient of the beta stabilising elements molybdenum and vanadium, about 45%, should be present in the alloy to give a useful level of creep resistance, the upper limit of the amounts in the alloy being set by considerations of both density and rate of oxidation, since molybdenum has a density of about twice that of titanium. Above about 50% total molybdenum and vanadium, any advantage that is derived from increased strength is offset by increased density. Moreover, the rate

2

of oxidation of these alloys increases rapidly as their titanium content is decreased below 50%.

Alloys containing molybdenum and vanadium in the proportions herein described provide a basic composition possessing a stable all-beta structure having good creep properties and room temperature strength with adequate ductility, as can be seen from Table II. This basic composition can be further improved by the addition of boron, particularly in respect of stress rupture. The following example demonstrates the effect of boron.

### Example I

120 gm. buttons of the alloys Ti-25 Mo-25 V and Ti-25 Mo-25 V-0.1 B were melted under argon in a non-consumable arc furnace using a tungsten electrode. The buttons were hammer forged to  $\frac{3}{4}$  inch square bar at 1200° C. and rod rolled to  $\frac{1}{2}$  inch square bar from a furnace at 1150° C. Stress rupture specimens were machined from the bars after they had been heated for 30 minutes at 900° C. and air-cooled. A life of 137 hours in stress rupture test at 25 tons/sq. in. at 600° C. is obtained with boron. The alloy without boron had a life of only half this under the same test conditions.

Strengthening of titanium by a dispersion of hard carbides is only possible when the matrix is stabilised by the presence of large amounts of beta promoters in the manner specified herein, otherwise the dispersion is unstable in favour of titanium carbide which is a relatively ineffective hardener at high temperatures. In a Ti-Mo-V base of the type described above, hafnium and carbon combine to form a finely divided dispersion of carbides which appreciably strengthens the alloy when in use at temperatures between 500 and 600° C.

The improvements in properties brought about separately by boron and by dispersion hardening can be incorporated into an alloy and thus results in a combination of good tensile properties at room temperature, excellent strength at temperatures between 500 and 600° C. and adequate ductility.

### Example II

A 5-pound ingot of the alloy Ti-25 Mo-25 V-2 Hf-0.1 C-0.1 B was vacuum arc cast using a consumable electrode. The ingot was machined to approximately 2 inches diameter and extruded to 1 inch diameter at 1200° C. The 1 inch diameter rod was re-extruded to  $\frac{1}{2}$  inch diameter at temperatures between 1000 and 1200° C. Tensile and stress-rupture test-pieces were machined from the rod after heating for 1 hour at 900° C. and air-cooling.

#### Room temperature tensile test:

|                        |   |        |      |
|------------------------|---|--------|------|
| 0.1% PS                | — | t.s.   | 67.7 |
| U.T.S.                 | — | t.s.i. | 73.5 |
| Percent elong. on 4V/A | — | —      | 31   |
| Percent R.A.           | — | —      | 36   |

#### Creep tests:

|                      |   |                                  |
|----------------------|---|----------------------------------|
| 20 t.s.i. at 550° C. | — | 0.02% total strain in 100 hours. |
| 20 t.s.i. at 575° C. | — | 0.06% total strain in 100 hours. |
| 10 t.s.i. at 600° C. | — | 0.1% total strain in 100 hours.  |

A basic composition containing 20% molybdenum and 20% vanadium is, however, preferred and alloys having this composition have been studied in greater detail and are discussed below.

The effect of zirconium, tantalum, tungsten and chromium on total strain in the first five hours of the stress rupture test are shown in Table III. Experience has shown that the creep strength of the alloys can be judged from such figures with reasonable accuracy. The carbon is also varied in alloys in the table and, whilst zirconium and tungsten improve strength, tantalum appears to have little or no effect.

Additions of carbon and boron both in the presence of

and in the absence of hafnium are shown in FIGURE 1 in which the basic composition is Ti-20 Mo-20 V and is stress rupture tested at 30 tons/sq. in. at 600° C. It will be seen that hafnium increases stress rupture life considerably and carbon and boron alone produce the best results. In FIGURE 2 the effects of various amounts of hafnium, carbon and boron are shown on the stress rupture life of Ti-20 Mo-20 V tested at 20 tons/sq. in. at 575° C. In general, increase in the amounts of these three elements increases the life.

Of the range of alloys herein disclosed, the preferred compositions are Ti-20 Mo-20 V-2 Hf-5 W-0.2 B and Ti-20 Mo-20 V-2 Hf-5 W-0.03 C-0.03 B and Ti-20 Mo-20 V-2 Hf-4 Zr-0.03 C. These alloys combine good creep strength and ductility with good fabricability.

TABLE I.—EFFECT OF ALLOYING ELEMENTS ON THE STRESS-RUPTURE LIFE OF Ti-20 Mo-20 V TESTED AT 20 T.S.I. AT 600° C.

| Alloy composition (wt. percent) | Stress-rupture life (hours) | Elongation percent |
|---------------------------------|-----------------------------|--------------------|
| Ti-20 Mo-20 V                   | 7.8                         | 33                 |
| Ti-20 Mo-20 V-9 W               | 77                          | 10                 |
| 2 Nb                            | 10                          | 28                 |
| 5 Nb                            | 22                          | 26                 |
| 1 Mn                            | 13                          | 10                 |
| 0.5 Zr                          | 7.5                         | 18                 |
| 1 Cr                            | 11                          | 31                 |
| 1 Ni                            | 3                           | 36                 |
| 1 Fe                            | 15                          | 26                 |
| 0.25 Hf                         | 10                          | 35                 |
| 0.5 Si                          | 11                          | 41                 |
| 0.5 Al                          | 6                           | 38                 |
| 1.5 Al                          | 10                          | 40                 |
| 0.25 B                          | 9                           | 31                 |

We claim:

1. A titanium-base alloy having high creep strength consisting essentially of 15-35% molybdenum, 15-35% vanadium, the total molybdenum plus vanadium content being in the range 40-55%, 0.01-0.2% boron, 0.1-5% hafnium, 0.01-0.2% carbon and the balance titanium apart from impurities said alloy being characterized by containing a fine dispersion of hafnium carbide.
2. A titanium-base alloy according to claim 1 containing in addition up to 8% zirconium.
3. A titanium-base alloy according to claim 2 containing in addition 4-8% zirconium.
4. A titanium-base alloy according to claim 2 containing in addition up to 5% zirconium.
5. A titanium-base alloy according to claim 1 containing in addition up to 10% tungsten, up to 5% tantalum, niobium, chromium and aluminium.
6. A titanium-base alloy according to claim 5 containing up to 5% tungsten.
7. A titanium-base alloy having high creep strength consisting of 25% molybdenum, 25% vanadium, 2% hafnium, 0.1% carbon, 0.1% boron, balance titanium and impurities, said alloy being characterized by containing a fine dispersion of hafnium carbide.
8. A titanium-base alloy having high creep strength consisting of 20% molybdenum, 20% vanadium, 2% hafnium, 5% tungsten, 0.03% carbon, 0.03% boron, balance titanium apart from impurities, said alloy being characterized by containing a fine dispersion of hafnium carbide.

TABLE II.—HOT HARDNESS AND STRESS-RUPTURE LIFE AT 600° C. OF Ti-Mo-V ALLOYS CONTAINING UP TO 50% BY WEIGHT OF (Mo+V)

| Button number | Composition, percent |       | Density, gm./cc. | Hardness value (D.P.N.) |         |         |         |                        |         |         |       | Stress rupture test, 600° C. |                                    |  |
|---------------|----------------------|-------|------------------|-------------------------|---------|---------|---------|------------------------|---------|---------|-------|------------------------------|------------------------------------|--|
|               | Mo                   | V     |                  | Increasing temperature  |         |         |         | Decreasing temperature |         |         |       | Life under 25 t.s.i. (hrs.)  | Elong. percent on 1st gauge length |  |
|               |                      |       |                  | R.T.                    | 500° C. | 600° C. | 700° C. | 700° C.                | 600° C. | 500° C. | R.T.  |                              |                                    |  |
| H189          | 30                   | 4.86  | 229              | 130                     | 79      | -----   | -----   | 79                     | 132     | 227     | ----- | 5.0                          | 31.3                               |  |
| H415          | 45                   | 5.07  | 314              | 234                     | 174     | 119     | 122     | 194                    | 242     | 327     | ----- | 5.0                          | 36.5                               |  |
| H416          | 50                   | 5.14  | 288              | 207                     | 172     | 112     | 108     | 185                    | 225     | 301     | ----- | 0.5                          | 36.5                               |  |
| H413          | 5                    | 40    | 5.16             | -----                   | -----   | -----   | -----   | -----                  | -----   | -----   | ----- | -----                        | -----                              |  |
| H414          | 5                    | 45    | 5.23             | 294                     | 218     | 171     | 117     | 117                    | 184     | 224     | 303   | 7.0                          | 42.6                               |  |
| H411          | 10                   | 35    | 5.25             | 305                     | 242     | 151     | 98      | 83                     | 149     | 240     | 308   | 3.5                          | 34.6                               |  |
| H412          | 10                   | 40    | 5.33             | -----                   | -----   | -----   | -----   | -----                  | -----   | -----   | ----- | (1)                          | -----                              |  |
| H227          | 15                   | 10    | 5.04             | 356                     | 202     | 105     | -----   | 103                    | 190     | 362     | ----- | -----                        | -----                              |  |
| H228          | 15                   | 15    | 5.11             | 358                     | 228     | 140     | -----   | 131                    | 202     | 321     | ----- | 0.75                         | 16.2                               |  |
| H286          | 15                   | 20    | 5.19             | 329                     | 215     | 134     | 86      | 88                     | 150     | 225     | 342   | 2.25                         | 29.1                               |  |
| H287          | 15                   | 25    | 5.26             | 288                     | 210     | 150     | 81      | 84                     | 160     | 230     | 327   | 10.0                         | 28.9                               |  |
| H366          | 15                   | 30    | 5.33             | 312                     | 296     | 247     | -----   | 255                    | 284     | 331     | 325   | 35.0                         | 23.2                               |  |
| H367          | 15                   | 35    | 5.40             | 323                     | 244     | 204     | -----   | 212                    | 233     | 212     | 289   | -----                        | -----                              |  |
| H229          | 20                   | 5     | 5.13             | 287                     | 190     | 143     | -----   | 140                    | 185     | 212     | 310   | -----                        | -----                              |  |
| H230          | 20                   | 10    | 5.20             | 333                     | 225     | 150     | -----   | 159                    | 212     | 212     | 212   | 0.6                          | 27.2                               |  |
| H288          | 20                   | 15    | 5.28             | 435                     | 290     | 200     | 75      | 103                    | 179     | 280     | 418   | 2.25                         | 20.7                               |  |
| H289          | 20                   | 20    | 5.36             | 312                     | 230     | 180     | 123     | 123                    | 225     | 270     | 378   | 8.0                          | 13.8                               |  |
| H368          | 20                   | 25    | 5.43             | 305                     | 234     | 194     | -----   | 167                    | 228     | 314     | 343   | 37.0                         | 27.4                               |  |
| H369          | 20                   | 30    | 5.51             | 347                     | 285     | 252     | -----   | 252                    | 279     | 343     | 328   | -----                        | -----                              |  |
| H231          | 25                   | 5     | 5.29             | 339                     | 234     | 166     | -----   | 168                    | 240     | 351     | 1.0   | 20.0                         | -----                              |  |
| H290          | 25                   | 10    | 5.37             | 366                     | 235     | 154     | 91      | 97                     | 152     | 210     | 355   | 5.0                          | 19.9                               |  |
| H291          | 25                   | 15    | 5.45             | 343                     | 235     | 175     | 116     | 124                    | 192     | 240     | 349   | 31.25                        | 14.7                               |  |
| H370          | 25                   | 20    | 5.53             | 352                     | 282     | 244     | -----   | 228                    | 273     | 303     | 280   | 70.0                         | 22.4                               |  |
| H371          | 25                   | 25    | 5.61             | 285                     | 202     | 145     | -----   | 153                    | 198     | 212     | 212   | 13.0                         | 15.0                               |  |
| H177          | 30                   | ----- | 5.39             | 275                     | 169     | 122     | -----   | 122                    | 166     | 212     | 325   | 20.25                        | 6.3                                |  |
| H372          | 30                   | 15    | 5.61             | 325                     | 231     | 174     | -----   | 212                    | 244     | 325     | 325   | -----                        | -----                              |  |
| H373          | 30                   | 20    | 5.69             | -----                   | -----   | -----   | -----   | -----                  | -----   | -----   | ----- | -----                        | -----                              |  |

<sup>1</sup> Flaws revealed on machining.

TABLE III.—TOTAL STRAIN IN THE FIRST 5 HOURS OF THE STRESS-RUPTURE TEST FOR VARIOUS ALLOYS BASED ON Ti-20 Mo-20 V-2 Hf TESTED AT 20 T.S.I. AT 575° C.

| Ti                     | Mo | V  | Hf | Zr    | W     | Ta    | Cr    | C    | B    | Total strain, ins./ins. in 5 hours |
|------------------------|----|----|----|-------|-------|-------|-------|------|------|------------------------------------|
| Balance in each alloy. | 20 | 20 | 2  | ----- | ----- | ----- | ----- | 0.03 | 0.1  | 0.0024                             |
|                        | 20 | 20 | 2  | ----- | ----- | ----- | ----- | 0.03 | 0.1  | 0.01                               |
|                        | 20 | 20 | 2  | ----- | 5     | ----- | ----- | 0.03 | 0.2  | 0.002                              |
|                        | 20 | 20 | 2  | ----- | 5     | ----- | 5     | 0.03 | 0.2  | 0.0014                             |
|                        | 20 | 20 | 2  | ----- | 5     | ----- | 5     | 0.03 | 0.03 | 0.0005                             |
|                        | 20 | 20 | 2  | ----- | 5     | ----- | 5     | 0.03 | 0.03 | 0.0027                             |
|                        | 20 | 20 | 2  | 4     | ----- | ----- | ----- | 0.03 | 0.03 | 0.0004                             |
|                        | 20 | 20 | 2  | ----- | ----- | ----- | ----- | 0.03 | 0.03 | 0.007                              |
|                        | 20 | 20 | 2  | ----- | ----- | ----- | ----- | 0.03 | 0.03 | 0.012                              |

9. A titanium-base alloy having high creep strength consisting essentially of 20% molybdenum, 20% vanadium, 2% hafnium, 4% zirconium, 0.03% carbon, balance essentially titanium apart from impurities said alloy being characterized by containing a fine dispersion of 5 hafnium carbide.

10. A titanium-base alloy as in claim 1 wherein the total molybdenum plus vanadium content is in the range 45-50%.

**References Cited**

10

**UNITED STATES PATENTS**

2,596,489 5/1952 Jaffee et al. ----- 75-175.5

|           |        |                    |          |
|-----------|--------|--------------------|----------|
| 2,819,960 | 1/1958 | Bomberger -----    | 75-175.5 |
| 2,938,789 | 5/1960 | Jaffee -----       | 75-175.5 |
| 3,306,739 | 2/1967 | Evans et al. ----- | 75-175.5 |

**OTHER REFERENCES**

"Development of a Ti-Al-Cb Alloy for Use at 1200-1800° F.", Armour Research Foundation, March 1962, 36 pages.

CHARLES N. LOVELL, *Primary Examiner.*